

May 17, 1932.

N. B. PILLING

1,858,415

ALLOY

Filed Sept. 23, 1924



WITNESSES:

Carl J. Loesch  
W.C. Wheeler.

INVENTOR

Norman B. Pilling  
BY  
Berkeley G. Carr  
ATTORNEY

## UNITED STATES PATENT OFFICE

NORMAN B. PILLING, OF PLAINFIELD, NEW JERSEY, ASSIGNOR TO WESTINGHOUSE ELECTRIC & MANUFACTURING COMPANY, A CORPORATION OF PENNSYLVANIA

## ALLOY

Application filed September 23, 1924. Serial No. 739,260.

My invention relates to alloys, more particularly to materials adapted for use in electrical instruments.

It is desirable in many cases to provide a resistor material for use in electrical instruments that has a negative temperature coefficient of resistance in order to compensate for the positive temperature coefficient of a part of the instrument. To accomplish this result there has been proposed an alloy of nickel and copper, which has a negative temperature coefficient and is known as "negatan". This material, which consists of 50% nickel and the remainder copper, with sometimes the addition of very small amounts of magnesium, has a relatively low negative temperature coefficient of resistance, usually about .00012, per degree centigrade but varying somewhat according to the conditions of manufacture. Furthermore, this material has a high thermo-electric power against copper.

It is among the objects of my invention to provide an alloy having a high negative temperature coefficient of resistance and having a low thermo-electric power against copper.

In practicing my invention, I have studied substantially the entire series of alloys, including copper, nickel and manganese as the principal constituents thereof, and have found that there is a region extending over a considerable range of amounts of the alloying ingredients in which the temperature coefficient is negative and is relatively high—much higher than that of negatan. I have further found that the alloys having the highest negative coefficients have relatively high resistivities, which is of great advantage in materials for compensation purposes in electrical instruments.

The accompanying drawing is a diagram showing the temperature coefficients of various alloys that I have studied and indicating the regions of equal coefficients. The figures denoting each of the regions should be multiplied  $10^{-4}$  to obtain the correct value of the temperature coefficient.

Referring to the figure, it will be found that the addition of nickel to copper rapidly lowers the coefficient until at 33% nickel con-

tent, it is zero; the addition of copper to nickel likewise reduces the coefficient to zero at 58% nickel content; the intermediate alloys have negative coefficients, with a minimum at about 50% nickel (negatan). 55

The addition of manganese up to 10% to the copper-nickel series has a marked effect. When the nickel content is below 28%, manganese rapidly decreases the coefficient, but above this content, up to 70% nickel, it causes 60 an increase in the coefficient, passing through a maximum at about 5% manganese, beyond which the coefficient decreases again. This condition has several peculiar results in that a zone of high coefficient alloys is found in 65 those containing about 30% copper and 5% manganese.

When manganese is added to copper, the coefficient is very rapidly decreased, reaching nearly zero at about 10% manganese, 70 passing through a flat minimum and rising again at 30% manganese. The temperature-resistance curve of copper manganese alloys in this range is not linear, but passes through a maximum, so that a given alloy may have 75 a positive, or negative coefficient depending on the temperature interval through which it is measured. The map of this region cannot therefore be very closely defined. Managanin is an alloy of this type in which a zero 80 coefficient is had by modifying the maximum on the curve so that it occurs at room temperature.

The first 10% of nickel added to copper-manganese alloys is without appreciable effect on the coefficient. 85

Manganese added to nickel reduces the coefficient at first relatively slowly, but passing through a minimum in the negative coefficient field with between 50 and 60% manganese content. A zero coefficient results at 40% manganese. Copper up to 10% added to the nickel-manganese group is without effect on the coefficient until manganese exceeds 15%, but beyond this range, copper first increases the coefficient and then causes it to decrease slowly. 90

The manganese corner has not been worked out, no alloys of more than 70% manganese having been made. In the interior of the 100

diagram, the coefficients first sink to zero and then below a great field of negative coefficient alloys occurs, forming at least half the area of the diagram. There are two negative fields that have been discovered. The first is that peculiar to the pure nickel-coppers, rapidly eliminated by an addition of manganese, and hence forming a narrow zone along the copper nickel base. Second, the great interior field, which connects with the nickel-manganese base line; its limits in the direction of the manganese corner have not been traced. The maximum negative coefficient is not found at equi-atomic proportions of copper, nickel and manganese, but at 10% removed from that condition. This alloy has a composition of about:

|           | Per cent |
|-----------|----------|
| Copper    | 24       |
| Nickel    | 36       |
| Manganese | 40       |

with a temperature coefficient of  $-.00032$  per  $1^{\circ}\text{C}$ .

The term "manganese" refers to the product known as pure manganese, which at the present stage of the metallurgical art, contains about 95% of manganese. Other elements present include about 1.7% iron and 1.5% silicon. It is apparent that all my alloys contain the latter elements in amounts proportional to the nominal content of manganese, and such proportional impurities will be understood herein in all instances where the content of manganese is specified.

It will be noted that I have produced an entirely new series of alloys having high negative temperature coefficients of resistance and a low thermo-electric power against copper which alloys are workable at room temperature and are malleable at elevated temperatures. The negative temperature coefficients of resistance of my new alloys are as high as four times that of negatan and the most malleable of such alloys has twice the temperature coefficient thereof. My alloys have a high resistivity compared to negatan and are, therefore, much more suitable for use in electrical instruments than the said material.

In my copending application, Serial No. 736,827 filed Sept. 10, 1924, for alloys, I have described and claimed alloys of the same three metals but having zero temperature coefficients, high resistivities and low thermo-electric power against copper.

I claim as my invention:

1. An alloy comprising 15% to 55% copper, less than 47% and more than 22% nickel and more than 20% manganese, said alloy having a negative temperature coefficient of resistance greater than  $1 \times 10^{-4}$  per degree centigrade.

2. An alloy comprising 5% to 49% copper, more than 22% and less than 45% nickel and more than 20% manganese, said alloy having

a negative temperature coefficient of resistance greater than  $1.5 \times 10^{-4}$  per degree centigrade.

3. An alloy comprising 5% to 45% copper, 25% to 45% nickel and less than 60% and more than 25% manganese, said alloy having a negative temperature coefficient of resistance greater than  $2 \times 10^{-4}$  per degree centigrade.

4. An alloy comprising 15% to 38% copper, 32% to 42% nickel and from 28% to 48% manganese, said alloy having a negative temperature coefficient of resistance greater than  $2.5 \times 10^{-4}$  per degree centigrade.

5. An alloy comprising 18% to 28% copper, 33% to 38% nickel and from 44% to 36% manganese, said alloy having a negative temperature coefficient of resistance greater than  $3 \times 10^{-4}$  per degree centigrade.

6. An alloy comprising approximately 24% copper, 36% nickel and 40% manganese.

In testimony whereof, I have hereunto subscribed my name this second day of September 1924.

NORMAN B. PILLING.

90

95

100

105

110

115

120

125

130